

Patented Nov. 9, 1926.

1,606,159

# UNITED STATES PATENT OFFICE.

COLIN G. FINK AND LI CHI PAN, OF NEW YORK, N. Y., ASSIGNORS TO CHEMICAL TREATMENT COMPANY, INC., OF NEW YORK, N. Y., A CORPORATION OF NEW YORK.

## PROCESS OF PRODUCING PROTECTIVE AND RESISTANT COATINGS.

No Drawing.

Application filed December 18, 1925. Serial No. 76,312.

This invention relates to processes of producing protective and resistant coatings, and aims to provide improvements therein.

Fink (one of the present applicants) and associates have heretofore produced resistant and protective coatings composed in whole or in part of chromium, and have devised several kinds of said coatings and several processes of producing the same. The 10 present invention is the result of the continuation of their investigations in this direction, having for object to produce a protective and resistant coating, having excellent qualities, by an economical and readily 15 performed procedure.

The present invention accordingly provides an improved process of producing coatings having excellent protective and resistant properties (that is, resistance to corrosion, acids, wear), which process is carried out in readily performed operations, resulting in an economical production of the coatings. The process further enables one to obtain bright coatings notwithstanding the use 25 of heat at elevated temperatures, and the susceptibility of the plated metal to oxidation and discoloration at the elevated temperature, when exposed to air.

According to the present invention, a foundation metal, as for example iron, steel, etc., is coated with chromium, preferably by electrodeposition. This coating may be from  $\frac{1}{2}$  mill to 1 mill thick, and may be produced according to the method of plating set forth 30 in the application of Fink and Eldridge filed August 26, 1924, Serial No. 734,193, and other applications of Fink and associates.

After plating, the metal article having thereon the plate is, without the necessity for 40 preparatory treatment, immersed in a bath of molten lead. This bath of lead is preferably maintained at a temperature somewhat above its melting point, a temperature of 800 C. being employed in practice.

The article is allowed to remain in the bath 45 of lead until it reaches the temperature of the bath, and preferably somewhat longer. The time will vary with the size and shape of the articles. With small articles having 50 about 24 square inches surface, and weighing about 4 ounces, the time of immersion is from one to two hours.

The heating of the article has the effect of 55 eliminating "pin-hole" defects in the chromium plate, producing a "healing" of these

defects, and probably produces a limited alloying of the chromium plate with the underlying foundation metal.

After the plated article has been sufficiently heat treated in the bath, it is removed therefrom.

After removal, the treated article has a film of lead adhering to the chromium plate. The surface of the chromium, however, is not discolored, and appears as a bright surface after removal of the lead film. This film of lead, where a bright non-tarnishing surface is desired, is then preferably removed, and this removal may be effected in a variety of ways. It may be conveniently effected by abrasion, inasmuch as chromium is very much harder than lead, and abrasives may be used which will readily attack the lead but will not affect the chromium. For example, a so-called scratch-brush may be used over the surface to remove the lead. Moreover, the lead may be removed by acids, an acid being selected which is inactive toward chromium and active toward lead, as for example, nitric acid.

The removal of lead by acid is preferably also employed after a treatment of the lead film by other methods. For instance, after the scratch-brush has been used upon the article, it is preferably dipped in nitric acid 55 in order to remove the last traces of lead, and with the lead completely removed the chromium surface is left without any substance thereon which would tarnish or darken, and thereby defeat the effect of a 60 bright, non-tarnishing surface which may be obtained with chromium.

The foregoing process may be used to advantage in producing bright resistant coatings of metals other than chromium, as for 65 example nickel.

The invention may be carried out by other modes of procedure than that herein specifically described.

What is claimed is:—

1. A method of producing protective and 70 resistant coatings of metals which are discolored and oxidized when heated in air, comprising plating a foundation-metal with the protective metal, and immersing the 75 plated metal article in a molten bath of lead to eliminate "pin-hole" defects in said plate by heat-treatment, without producing discoloration of said protective metal.

2. A method of producing protective and 80

- resistant coatings of metals which are discolored and oxidized when heated in air, comprising plating a foundation-metal with the protective metal, and immersing the plated metal article in a molten bath of lead to eliminate "pin-hole" defects in said plate by heat-treatment, without producing discoloration of said protective metal, and removing the film of lead remaining on the plate after removal from the bath.
3. A method of producing protective and resistant coatings of metals which are discolored and oxidized when heated in air, comprising plating a foundation-metal with the protective metal, and immersing the plated metal article in a molten bath of lead to eliminate "pin-hole" defects in said plate by heat-treatment, without producing discoloration of said protective metal, and removing by abrasion the film of lead remaining on the plate after removal from the bath.
4. A method of producing protective and resistant coatings of metals which are discolored and oxidized when heated in air, comprising plating a foundation-metal with the protective metal, and immersing the plated metal article in a molten bath of lead to eliminate "pin-hole" defects in said plate by heat-treatment, without producing discoloration of said protective metal, and removing by acid the film of lead remaining on the plate after removal from the bath.
5. A method of producing protective and

resistant coatings of metals which are discolored and oxidized when heated in air, comprising plating a foundation-metal with the protective metal, and immersing the plated metal article in a molten bath of lead to eliminate "pin-hole" defects in said plate by heat-treatment, without producing discoloration of said protective metal, and removing by abrasion and acid the film of lead remaining on the plate after removal from the bath.

6. A method of producing protective and resistant bright coatings of chromium, comprising plating a foundation-metal with chromium, immersing the chromium-plated article in a molten bath of lead to eliminate "pin-hole" defects in said plate by heat-treatment, without producing discoloration of said chromium plate.

7. A method of producing protective and resistant bright coatings of chromium, comprising plating a foundation-metal with chromium, immersing the chromium-plated article in a molten bath of lead to eliminate "pin-hole" defects in said plate by heat-treatment, without producing discoloration of said chromium plate, and removing the film of lead remaining on the plate after removal from the bath.

In witness whereof, we have hereunto signed our names.

COLIN G. FINK.  
LI C. PAN.